

Nov. 25, 1958

C. G. MICKELSON ET AL

2,861,908

ALLOY STEEL AND METHOD OF MAKING

Filed Nov. 30, 1955

8 Sheets-Sheet 1



Inventors:  
Gustaf A. Lillieqvist  
Cedric G. Mickelson  
By: Walter L. Schlegel, Jr. Atty.

Nov. 25, 1958

C. G. MICKELSON ET AL

2,861,908

ALLOY STEEL AND METHOD OF MAKING

Filed Nov. 30, 1955

8 Sheets-Sheet 2



Inventors:  
Gustaf A. Lilliequist  
Cedric G. Mickelson  
By: Walter L. Schlegel, Jr. Atty.

Nov. 25, 1958

C. G. MICKELSON ET AL  
ALLOY STEEL AND METHOD OF MAKING

2,861,908

Filed Nov. 30, 1955

8 Sheets-Sheet 3

Fig. 3.



Inventors:  
Gustaf A. Lillqvist  
Cedric G. Mickelson  
By Walter L. Schlegel, Jr. Atty.

Nov. 25, 1958

C. G. MICKELSON ET AL

2,861,908

ALLOY STEEL AND METHOD OF MAKING

Filed Nov. 30, 1955

8 Sheets-Sheet 4

Fig. II.



Inventors

Gustaf A. Lillieqvist  
Cedric G. Mickelson

By Walter L. Schlegel, Jr. Atty.

Nov. 25, 1958

C. G. MICKELSON ET AL

2,861,908

ALLOY STEEL AND METHOD OF MAKING

Filed Nov. 30, 1955

8 Sheets-Sheet 5

*Fig. 5*



*Fig. 6*



INVENTORS  
*Gustaf A. Lillqvist*  
BY *Cedric G. Mickelson*  
*Walter S. Schlegel, Jr.*  
*Otti*

Nov. 25, 1958

C. G. MICKELSON ET AL

2,861,908

ALLOY STEEL AND METHOD OF MAKING

Filed Nov. 30, 1955

8 Sheets-Sheet 6

Fig. 7



Inventors:  
Gustaf A. Lilliequist  
Cedric G. Mickelson  
By: Walter L. Schlegel, Jr. Atty.

Nov. 25, 1958

C. G. MICKELSON ET AL

2,861,908

ALLOY STEEL AND METHOD OF MAKING

Filed Nov. 30, 1955

8 Sheets-Sheet 7

*Fig. 8*



Inventors,  
Gustaf A. Lillieqvist  
Cedric G. Mickelson

By: *Walter L. Schlegel, Jr.* Atty.

Nov. 25, 1958

C. G. MICKELSON ET AL

2,861,908

ALLOY STEEL AND METHOD OF MAKING

Filed Nov. 30, 1955

8 Sheets-Sheet 8

Fig. 9.



Inventors:  
Gustaf A. Lilliequist  
Cedric G. Mickelson  
By: Walter L. Schlegel, Jr. Atty.

# United States Patent Office

2,861,908

Patented Nov. 25, 1953

1

2,861,908

## ALLOY STEEL AND METHOD OF MAKING

Cedric G. Mickelson, Gary, Ind., and Gustaf A. Lillieqvist, deceased, late of Hammond, Ind., by Ellen S. Lillieqvist, administratrix, Lake County, Ind., assignors to American Steel Foundries, Chicago, Ill., a corporation of New Jersey

Application November 30, 1955, Serial No. 549,910

15 Claims. (Cl. 148—31)

This invention relates to alloy steels and to a method of manufacturing and heat treating them, and more particularly to alloy steel castings having improved wear resistance and toughness. This application is a continuation-in-part of our copending application, Serial No. 451,652, filed on August 23, 1954, now abandoned.

There has been a long felt need for a tough steel alloy having great resistance to wear without tendency to deform. For example, in the production of cast steel parts, such as dipper buckets or dipper teeth, which are subjected to frequent and severe abrasion as well as blows of substantial magnitude, wear resistance and toughness, without tendency to deform, are of extreme importance.

Ordinary steels used in the production of such parts have not only been inadequate to resist wear but have in many cases tended to creep or deform from repeated use, as is normally encountered in service.

According to the present invention, an alloy steel has been discovered containing rare earth metals and boron added in the molten state, which when normalized, hardened, and tempered by heating to a temperature less than 600° F., followed by a quench, is astonishingly tough and resistant to wear, without tendency to deform in service.

It has been found that the novel steel alloy after heat treatment is characterized by a fine grain micro-structure predominantly in the form of tough interlocked martensitic needles and is characterized by a Brinell hardness value of 400 or more and by a Charpy impact value of 12 or more foot pounds at room temperature and 10 or more foot pounds at —40° F.

It has also been found that the novel steel is machineable at Brinell hardness values up to 515 and is unusually resistant to corrosion. The novel steel is also self hardening under service conditions which intermittently heat the steel to its upper critical temperature value.

The alloy steel of this invention may comprise broadly the following composition:

| Component         | Percent by Weight                                                                                 |
|-------------------|---------------------------------------------------------------------------------------------------|
| Carbon            | about .20 to .50%.                                                                                |
| Manganese         | about .70 to 1.70%.                                                                               |
| Silicon           | about .20 to 2.0%.                                                                                |
| Phosphorus        | nil to about .05%.                                                                                |
| Sulphur           | Do.                                                                                               |
| Molybdenum        | about .05 to 7.0%.                                                                                |
| Chromium          | about 0.5 to 1.50%.                                                                               |
| Nickel            | about .01 to 1.00%.                                                                               |
| Boron             | about .0005 to .005% added to the metal in the molten state.                                      |
| Rare Earth Metals | The residue from the treatment of the molten metal in the molten state with about 0.0015 to 0.5%. |
| Iron              | Balance with residual impurities in ordinary amounts.                                             |

2

It has also been discovered that an economical composition of the novel alloy limited to narrower ranges is particularly effective for certain applications, in which case the following concentrations of alloying elements will produce an alloy having the desirable characteristic of wear resistance:

| Component         | Percent by Weight                                                                                 |
|-------------------|---------------------------------------------------------------------------------------------------|
| Carbon            | about .20 to .50%.                                                                                |
| Manganese         | about .70 to 1.70%.                                                                               |
| Silicon           | about .20 to 2.0%.                                                                                |
| Phosphorus        | nil to about .05%.                                                                                |
| Sulphur           | Do.                                                                                               |
| Molybdenum        | about .05 to 7.0%.                                                                                |
| Chromium          | about 0.5 to 1.50%.                                                                               |
| Nickel            | about .01 to 1.00%.                                                                               |
| Boron             | about .0005 to .005% added to the metal in the molten state.                                      |
| Rare Earth Metals | The residue from the treatment of the molten metal in the molten state with about 0.0015 to 0.5%. |
| Iron              | Balance with residual impurities in ordinary amounts.                                             |

It may also be noted that titanium in an amount of the order of nil to 5 pounds per ton of charge may be added to the alloy in the molten state prior to addition of the boron and rare earths. Titanium is preferably added in the form of ferrotitanium although other forms thereof may be used. Under certain melting conditions it has been found that the addition of titanium is critical as, for example, when the steel is cast at a very high temperature or has been subjected to a long hold after having been killed in the furnace. Under these conditions nitrogen absorption by the steel may be very high. Also a heat having a poor boil may tend to have a high soluble nitrogen content. Under any one of these conditions titanium must be added to change the soluble nitrogen into an insoluble nitrogen compound, titanium nitride, which has been found to have no appreciable effect on the hardenability characteristics of the steel. Thus when the boron and rare earth additions are made subsequent to the titanium addition, the boron and rare earths pass into solid solution in the iron, whereas the boron might otherwise form boron nitride which would use up the boron and not allow it to alloy with the steel and produce the desired hardenability characteristics.

It has been discovered in this connection that the soluble nitrogen in the steel must not exceed about .008% when the rare earth and boron additions are made. Thus, the titanium addition is desirable, when the soluble nitrogen in the steel is .008% or more, to preserve the characteristics imparted to the alloy not only by the boron but by the rare earth addition as well.

It will be understood that the value of the titanium addition is in direct proportion to the amount of soluble nitrogen in the molten steel, and if melting conditions are such that the soluble nitrogen content is at a very low value, the titanium addition may be eliminated in the interest of economy. However, in any event, the titanium addition is preferred and has been found to improve the properties of the novel steel alloy to the extent that the titanium combines with soluble nitrogen. The effective range of titanium for the purpose is from about .0005 to about .02% by weight.

It has been found that a low carbon alloy steel such as above described having the desired characteristic of wear resistance and presenting minimum difficulties from

a viewpoint of heat treatment contains the following concentrations of alloying elements:

| Component         | Percent by Weight                                                                                |
|-------------------|--------------------------------------------------------------------------------------------------|
| Carbon            | about .26 to .30%.                                                                               |
| Manganese         | about 1.35 to about 1.55%.                                                                       |
| Silicon           | about .30 to .49%.                                                                               |
| Phosphorus        | nil to about .020%.                                                                              |
| Sulphur           | Do.                                                                                              |
| Molybdenum        | about .47 to .53%.                                                                               |
| Chromium          | about .52 to .68%.                                                                               |
| Nickel            | residual.                                                                                        |
| Rare Earth Metals | The residue from the treatment of the molten metal in the molten state with about .0015 to 0.5%. |
|                   | about .0020 to .005% added to the metal in the molten state.                                     |
| Boron             | Balance with residual impurities in ordinary amounts.                                            |
| Iron              |                                                                                                  |

A higher carbon alloy having even greater resistance to wear, but presenting certain difficulties from a viewpoint of the heat treatment, has been found to contain the following concentrations of alloying elements:

| Component         | Percent by Weight                                                                                |
|-------------------|--------------------------------------------------------------------------------------------------|
| Carbon            | about .33 to .37%.                                                                               |
| Manganese         | about 1.35 to 1.55%.                                                                             |
| Silicon           | about .30 to .49%.                                                                               |
| Phosphorus        | nil to about .020%.                                                                              |
| Sulphur           | Do.                                                                                              |
| Molybdenum        | about .47 to .53%.                                                                               |
| Chromium          | about .52 to .68%.                                                                               |
| Nickel            | residual.                                                                                        |
| Rare Earth Metals | The residue from the treatment of the molten metal in the molten state with about .0015 to 0.5%. |
|                   | about .0020 to .005% added to the metal in the molten state.                                     |
| Boron             | Balance with residual impurities in ordinary amounts.                                            |
| Iron              |                                                                                                  |

According to the invention, the novel steel alloy, after casting thereof, is heat treated in the following manner to achieve maximum wear resistance and toughness. The castings are first normalized by heating them, for example, to about 1600-1900° F. After a hold of any desired duration, the castings are then air cooled so that they may be conveniently worked in the shop. This treatment is followed by a hardening heat treatment in which the castings formed of the lower carbon steel alloy above mentioned are heated, for example, to about 1500-1700° F., and the higher carbon alloy steel castings are heated, for example, to about 1450-1650° F. In either case the castings are preferably held at the hardening temperature for about an hour or more, depending upon the section and are then quenched, preferably in water.

The castings are then heated to a tempering temperature of the order of 100° F. or more up to but less than 600° F., although unusually excellent results have been attained within a range of about 250 to 450° F. The castings are held at the tempering temperature, preferably for a period of about two hours or more depending upon the size of the castings and are then quenched, preferably in water, or possibly in air.

It will be understood that the hold time for the various heat treatments may vary considerably depending upon the type of furnace equipment and the size of material being produced. The shortest possible time at temperature is preferred, and it may be noted that excellent results have been achieved by the foregoing practice. If desired, in addition to the above described heat treatment, the castings may be tempered before hardening to reduce machining costs.

The term "rare earth metals" as used herein is intended to mean the following elements either singly or in combination: cerium, lanthanum, neodymium, praseodymium, samarium, illinium, europium, gadolinium, dysprosium, ytterbium, their alloys and compounds. These rare earth metals may be in the form of a mixture commonly known as "misch metal." A mixture of rare earth metals which has proved particularly effective contains about 31.5% lanthanum, about 44.5% cerium, about 11% praseodymium, about 7% neodymium and about 6% of the other rare earth metals above mentioned.

The percentage of rare earth metals and boron additions is critical and must be maintained substantially within the ranges set out above.

It is also noted that the tempering temperature is critical inasmuch as it has been discovered that brittleness of the castings is caused by tempering at a temperature of about 700° F., and wear resistance of the castings is inadequate if they are tempered at a temperature in excess of 700° F. Under certain conditions, the tempering step may be eliminated entirely, although this is not ordinarily desirable.

It has been found that in manufacturing the steel alloy of this invention, the molten steel is preferably killed in the furnace as, for example, by adding a deoxidizer such as aluminum, ferromanganese, ferrochrome, siliconmanganese and/or ferrosilicon. When the ladle is partly full, the steel is preferably further deoxidized, and then aluminum and titanium (if any) are preferably added, the aluminum being in an amount of the order of one to five pounds per ton of charge. The boron and rare earth elements are then added, irrespective of sequence; and finally an addition of calcium silicon is made, preferably in an amount of the order of three pounds per ton of charge before the ladle is completely filled.

If the steel is produced in small quantities, as, for example, in an induction furnace, the additions may be made in the furnace prior to pouring of the heat.

It has been further discovered that, within the ranges above specified, the alloying elements are effective only if the addition is made to molten steel in a basic condition, and it may be noted that the alloying elements may be added to the ladle as the basic steel is poured from the furnace; or if an acid lined furnace is used, the molten steel and slag may be poured into a first ladle wherein the slag may be converted to a basic condition, and the steel and slag may then be poured into a second ladle wherein the alloying additions are made.

The unusual properties of steel castings produced in the foregoing manner are best demonstrated by referring to tests of castings which were composed and heat treated within the specified ranges. The results of these tests are set forth in the tables which appear hereafter and in the accompanying drawings, wherein:

Figure 1 is a graph illustrating the effect of tempering temperatures on the toughness of the novel steel alloy casting (about .25% carbon) at room temperature;

Figure 2 is a graph illustrating the effect of tempering temperatures on the toughness of the same steel alloy castings at low temperatures of the order of -40° F.;

Figure 3 is a graph comparing the relationship between hardness and low temperature toughness of the same steel alloy castings with those of substantially identical steel alloy castings produced in the same manner but lacking the rare earth metals;

Figure 4 is a graph illustrating the effect of tempering temperatures on the hardness of the same steel alloy castings;

Figure 5 shows the microstructure of the novel steel alloy castings illustrated by the graphs of Figures 1-4;

Figure 6 shows the microstructure of a similar steel alloy casting tempered at a tempering temperature of the order of 1000° F. or more;

Figure 7 is a graph comparing the toughness of the novel steel alloy castings (about .26% carbon) with those of substantially identical steel castings produced and heat treated in the same manner but lacking either boron or rare earth metals;

Figure 8 is a graph showing the effect of tempering temperatures on the physical characteristics of the novel steel alloy castings containing about .30% carbon;

Figure 9 is a graph showing the effect of tempering temperatures on the physical characteristics of the novel steel alloy castings containing about .25% carbon and about 1.0% chromium and nickel.

Specific examples are disclosed as follows:

*Example No. 1*

Two heats were poured with the following analyses:

| Heat No. | C   | Mn   | Si  | P    | S    | Cr  | Mo  | Ni  | B     |
|----------|-----|------|-----|------|------|-----|-----|-----|-------|
| 7816     | .25 | 1.46 | .39 | .016 | .027 | .52 | .47 | .26 | .0024 |
| 7817     | .25 | 1.46 | .36 | .015 | .027 | .54 | .47 | .26 | .0024 |

| Block No. | Rockwell "C" Readings | Average Rockwell "C" Converted to Brinell |
|-----------|-----------------------|-------------------------------------------|
| 7816 AQ   | 47.5-48-47-47.5       | 472                                       |
| 7816 1    | 45-47.5-47.5-48       | 465                                       |
| 7816 2    | 46.5-48-47-47         | 465                                       |
| 7816 3    | 47-48-47-48.5         | 472                                       |
| 7816 4    | 47-47.5-45.5-47       | 458                                       |
| 7816 5    | 45.5-46-45.5-46       | 446                                       |
| 7816 6    | 44-45-44-45           | 434                                       |
| 7816 7    | 42-43-43-43.5         | 415                                       |
| 7816 8    | 40-40-39-40           | 385                                       |
| 7816 9    | 36.5-37-36-38         | 356                                       |
| 7816 10   | 34.5-34.5-34.5-35.5   | 333                                       |
| 7816 11   | 28-29-28-30           | 232                                       |
| 7816 12   | 21.5-23.5-20-24.5     | 244                                       |
| 7816 13   | 18-19-18.5-17         | 222                                       |
| 7817 AQ   | 47-47-44-45           | 446                                       |
| 7817 1    | 46.5-47-46.5-47       | 458                                       |
| 7817 2    | 46.0-46-48-47         | 458                                       |
| 7817 3    | 46-47.5-46-47         | 458                                       |
| 7817 4    | 45.5-47-45-47         | 452                                       |
| 7817 5    | 44.5-46-44-45.5       | 440                                       |
| 7817 6    | 43-44-43-44           | 421                                       |
| 7817 7    | 41-43-41.5-42         | 405                                       |
| 7817 8    | 39-40-39.5-40         | 380                                       |
| 7817 9    | 36-37-36-37           | 351                                       |
| 7817 10   | 35.5-34.5-32.5-34.5   | 329                                       |
| 7817 11   | 27.5-29.5-27-29       | 278                                       |
| 7817 12   | 46-46-49-49           | 238                                       |
| 7817 13   | 40-43-57-54           | 220                                       |

Charpy results at room temperature were as follows:

| Block No. | Charpy, Ft.-Lb. | Average | Brinell (From Rockwell "C") |
|-----------|-----------------|---------|-----------------------------|
| 7816 AQ   | 19-18-18-19     | 18.5    | 472                         |
| 7816 1    | 22-21-21-21     | 21      | 465                         |
| 7816 2    | 17-18-19-20     | 18.5    | 465                         |
| 7816 3    | 24-21-20-20     | 21      | 472                         |
| 7816 4    | 21-20-22-22     | 21      | 458                         |
| 7816 5    | 18-20-19-19     | 19      | 446                         |
| 7816 6    | 21-22-19-18     | 20      | 434                         |
| 7816 7    | 18-19-19-14     | 17.5    | 415                         |
| 7816 8    | 23-22-23-21     | 22      | 385                         |
| 7816 9    | 32-26-32-32     | 30.5    | 356                         |
| 7816 10   | 40-40-39-39     | 39.5    | 333                         |
| 7816 11   | 52-56-55-54     | 54      | 282                         |
| 7816 12   | 68-68-68-72     | 68.5    | 244                         |
| 7816 13   | 60-57-57-53     | 59      | 222                         |
| 7817 AQ   | 14-13-16-15     | 14.5    | 446                         |
| 7817 1    | 16-16-15-16     | 16      | 458                         |
| 7817 2    | 15-15-16-17     | 16      | 458                         |
| 7817 3    | 17-17-16-17     | 17      | 458                         |
| 7817 4    | 14-15-16-16     | 15      | 452                         |
| 7817 5    | 14-13-12-15     | 13.5    | 440                         |
| 7817 6    | 15-14-15-14     | 14.5    | 421                         |
| 7817 7    | 15-14-15-14     | 14.5    | 405                         |
| 7817 8    | 16-17-16-17     | 16.5    | 380                         |
| 7817 9    | 21-21-19-21     | 20.5    | 351                         |
| 7817 10   | 30-30-29-30     | 30      | 329                         |
| 7817 11   | 33-40-40-39     | 39      | 278                         |
| 7817 12   | 46-46-49-49     | 47.5    | 238                         |
| 7817 13   | 40-43-57-54     | 47.5    | 220                         |

Charpy results at -40° F. were as follows:

| Block No. | Charpy, Ft.-Lb. | Average | Brinell (From Rockwell "C") |
|-----------|-----------------|---------|-----------------------------|
| 7816 AQ   | 18-17-19-19     | 18      | 472                         |
| 7816 1    | 17-17-20-20     | 18.5    | 465                         |
| 7816 2    | 16-20-19-19     | 18.5    | 465                         |
| 7816 3    | 21-22-21-21     | 20.5    | 472                         |
| 7816 4    | 15-20-19-20     | 18.5    | 458                         |
| 7816 5    | 20-19-18-18     | 18      | 446                         |
| 7816 6    | 7-18-19         | 14.5    | 434                         |
| 7816 7    | 16-23-18-18     | 18.5    | 415                         |
| 7816 8    | 21-18-20-20     | 19.5    | 385                         |
| 7816 9    | 28-26-27-25     | 26.5    | 356                         |
| 7816 10   | 51-52-51-53     | 51.5    | 333                         |
| 7816 11   | 62-65-63-65     | 63.5    | 282                         |
| 7816 12   | 29-38-44-37     | 37      | 244                         |
| 7816 13   | 19-15-15-14     | 15.5    | 222                         |
| 7817 AQ   | 15-17-13-16     | 15      | 446                         |
| 7817 1    | 17-14-14-15     | 15      | 458                         |
| 7817 2    | 18-16-16-16     | 16.5    | 458                         |
| 7817 3    | 19-15-17-15     | 16.5    | 458                         |
| 7817 4    | 13-10-12-14     | 12      | 452                         |
| 7817 5    | 14-8-14-12      | 11      | 440                         |
| 7817 6    | 12-14-10-10     | 11.5    | 421                         |
| 7817 7    | 15-16-16-16     | 16      | 405                         |
| 7817 8    | 22-21-20-21     | 21      | 380                         |
| 7817 9    | 34-37-38-37     | 36.5    | 351                         |
| 7817 10   | 40-34-36-36     | 36.5    | 329                         |
| 7817 11   | 29-22-36-35     | 30.5    | 278                         |
| 7817 12   | 40-43-57-54     | 47.5    | 238                         |
| 7817 13   | 29-22-36-35     | 30.5    | 220                         |

After heat treatment the sections were machined into four Charpy specimens. Hardness readings taken on the tested Charpy specimens were as follows:

The graphs shown in Figures 1-4 were derived from the foregoing data and illustrate relationships found to exist with respect to tempering temperatures, toughness, hardness and addition practice.

Referring to Figure 1, it will be seen that a brittle zone resulted from a tempering temperature of the order of 700° F., in the case of the novel steel alloy containing rare earth elements and boron (Heat No. 7816) as illustrated by the top line in this graph. The sections heat treated at temperature values above 700° F. were found to have inadequate resistance to wear due to the low hardness values shown in Figure 4. Referring again to Figure 1, it will be seen that the best results with respect to toughness were achieved by tempering temperatures between 300 and 400° F., although very good results in this regard were attained by tempering temperatures below 600° F.

Referring to Figure 2, it will be seen that a low temperature brittle zone resulted from a tempering temperature of 700° F. in the case of the novel steel alloy containing rare earth elements and boron (Heat No. 7816) illustrated by the upper line of the graph. The best results in this regard resulted from tempering temperatures between 300 and 400° F., although good results were attained at temperatures below 600° F.

As illustrated by both graphs of Figures 1 and 2, the novel steel alloy (Heat No. 7816) was greatly superior from a viewpoint of toughness than that to which the rare earth elements were not added (Heat No. 7817).

Referring now to Figure 3, it will be seen that a brittle zone was discovered in the novel steel alloy (Heat No. 7816) at a Brinell hardness of approximately 415. At greater hardness values than 415, toughness increased, with the best results from this viewpoint at a Brinell hardness of 440 or greater.

Referring now to Figures 5 and 6, it will be seen that Figure 5 illustrates the microstructure of a casting composed of the novel steel alloy magnified 600 times. The steel alloy casting of Figure 5 is composed of Heat No. 7816 normalized and hardened as above described, and tempered at 375° F. It will be noted, as seen in Figure 5, that the microstructure is fine, predominately in the form of tough interlocked martensitic needles. The steel alloy casting shown in Figure 6 is also magnified 600 times, and it will be seen that the martensitic needles are no longer plainly visible in the microstructure of Figure 6 due to the fact that this casting was tempered at about 1000° F. or more. As a result the wear resistance of the steel alloy casting shown in Figure 6 is quite inferior to that of Figure 5.

#### Example No. 2

Referring now to Figure 7, which is a graph comparing the toughness of the novel steel alloy with that of substantially identical steels lacking either boron or the rare earth metals, it will be seen that the steel alloy of Heat No. 7718 which contained no boron was the least tough, and the steel alloy of Heat No. 7719 which contained no rare earth metals was less tough than that of Heat No. 7773 which contained both boron and the rare earth metals.

The following table compares the composition of these three heats:

| Heat No. | C   | Mn   | Si  | P    | S    | Cr  | Mo  | Ni  | B     |
|----------|-----|------|-----|------|------|-----|-----|-----|-------|
| 7773     | .26 | 1.35 | .34 | .015 | .027 | .51 | .50 | .25 | .0024 |
| 7719     | .26 | 1.38 | .25 | .016 | .027 | .50 | .50 | .24 | .0024 |
| 7718     | .26 | 1.32 | .28 | .016 | .027 | .52 | .49 | .25 |       |

Heat No. 7773 was treated in the molten state in accordance with the above described practice with 1½ pounds of aluminum per ton of charge, then 2 pounds of the rare earth metal mixture per ton of charge, then .0024% boron added in the form of "Borosil," and

finally 3 pounds of calcium-manganese-silicon per ton of charge.

Heat No. 7719 was treated in the molten state by adding 2½ pounds of aluminum per ton of charge, then .0024% boron added as "Borosil," and finally 3 pounds of calcium-manganese-silicon per ton of charge.

Heat No. 7718 was treated in the molten state by adding 1½ pounds of aluminum per ton of charge, then 2 pounds of the rare earth metal mixture per ton of charge, and finally 3 pounds of calcium-manganese-silicon per ton of charge.

All three of these heats were produced in basic lined induction furnaces, and the addition practice was identical except for the fact that the rare earth metal mixture was eliminated from Heat No. 7719 and boron was eliminated from Heat No. 7718.

Steel from these heats was poured into test runners from 1" x 6" x 10" Charpy blocks. All runners and the Charpy blocks were normalized at 1750° F. for 2 hours. The runners were machined into plugs and inserted into 5" Charpy blocks. All blocks were then hardened by heating to 1650° F., holding one hour and water quenching. The tempering treatments for the various blocks were as follows:

| Heat and Block No.        | Temperature, °F. | Hold, hours | Cooling       |
|---------------------------|------------------|-------------|---------------|
| 7773-1C, 7719-1C, 7718-1C | 1,000            | 2           | water quench. |
| 7773-1X, 7719-1X, 7718-1X | 1,050            | 2           | Do.           |
| 7773-1A, 7719-1A, 7718-1A | 1,100            | 2           | Do.           |
| 7773-2C, 7719-2C, 7718-2C | 1,100            | 2           | Do.           |
| 7773-2X, 7719-2X, 7718-2X | 1,165            | 2           | Do.           |
| 7773-2A, 7719-2A, 7718-2A | 1,210            | 2           | Do.           |
| 7773-5C, 7719-5C, 7718-5C | 1,120            | 2           | Do.           |
| 7773-5X, 7719-5X, 7718-5X | 1,185            | 2           | Do.           |
| 7773-5A, 7719-5A, 7718-5A | 1,250            | 2           | Do.           |
| 7773-8C                   | 1,120            | 2           | Do.           |
| 7773-8X                   | 1,185            | 2           | Do.           |
| 7773-8A                   | 1,260            | 2           | Do.           |
| 7719-8C                   | 1,120            | 2           | Do.           |
| 7719-8X                   | 1,185            | 2           | Do.           |

After final heat treatment, hardness readings were taken from slices of the 5 inch blocks as follows:

| Heat and Block No. | Rockwell "C" Readings Center to Surface           |
|--------------------|---------------------------------------------------|
| 7773-5C            | 27.5-28.0-29.0-29.0-29.0-29.0-29.0-30.0           |
| 45 7773-5X         | 29.5-30.0-30.0-30.0-30.5-30.0                     |
| 7773-5A            | 25.0-25.0-24.5-24.5-25.5-25.0-25.0-25.0-25.0      |
| 7719-5C            | 20.0-21.0-20.5-20.5-21.0-21.0-20.5-22.0-21.5-21.0 |
| 50 7719-5X         | 22.0-21.5-22.0-21.5-22.5-23.5-23.0-22.5           |
| 7719-5A            | 27.0-27.0-27.0-27.0-27.0-27.0-27.5-28.0-27.5      |
| 7719-5A            | 28.0-28.5-28.0-28.5-29.5-29.5-29.5                |
| 7719-5X            | 26.0-25.0-25.0-26.0-26.0-26.0-25.5-26.0-25.5      |
| 55 7719-5A         | 26.0-25.5-26.0-26.0-26.0-26.0-25.5-25.5           |
| 7718-5C            | 22.0-22.0-22.0-22.0-22.0-22.0-22.0-22.0-22.0      |
| 7718-5X            | 22.0-22.0-22.0-22.0-22.0-22.0-22.0-22.0-22.0      |
| 7718-5A            | 25.0-25.0-24.5-24.5-24.0-24.0-25.5-25.0-26.5      |
| 7718-5X            | 26.0-25.5-27.5-27.0-27.0-27.5-27.5-30.0           |
| 7718-5A            | 23.0-22.0-22.0-23.0-23.0-23.0-22.5-23.0-23.0      |
| 7718-5A            | 23.0-24.0-24.0-25.0-25.0-26.0-27.0-26.5           |
| 7718-5A            | 18.0-19.0-18.5-19.0-18.5-20.0-19.5-20.0-20.0      |
| 7718-5A            | 20.0-20.5-20.0-21.0-22.0-22.0-22.5-23.5-24.0      |

Charpy specimens were machined from the plugs and from the 5 inch Charpy blocks, and the results when tested at -40° F. were as follows:

| Heat and Block No. | Location of Notch   | Foot Pounds<br>-40° F. | Avg. | Average<br>Brinell |
|--------------------|---------------------|------------------------|------|--------------------|
| 7773-5C            | 1/16" from surface  | 50-51-54-54            | 53.4 | 287                |
| 7773-5X            | 2 1/2" from surface | 56-56-54-X             | 62.9 | 261                |
| 7773-5A            | 1/16" from surface  | 63-60-65-61            | 64   | 241                |
| 7773-5A            | 2 1/2" from surface | 64-62-64-64            | 69   | 279                |
| 7719-5C            | 1/16" from surface  | 69-69-67-70            | 70.3 | 258                |
| 7719-5X            | 2 1/2" from surface | 72-74-72-70            | 38.5 | 238                |
| 7719-5A            | 1/16" from surface  | 37-37-36-38            | 41.2 | 258                |
| 7719-5A            | 2 1/2" from surface | 43-43-43-43            | 42.6 | 229                |
| 70 7719-5A         | 1/16" from surface  | 44-44-43-45            | 44.0 | 238                |
| 7718-5C            | 1/16" from surface  | 22-23-23-25            | 20.0 | 272                |
| 7718-5X            | 2 1/2" from surface | 18-19-16-14            | 33.2 | 255                |
| 7718-5X            | 1/16" from surface  | 36-38-40-33            | 37   | 255                |
| 7718-5A            | 2 1/2" from surface | 39-48-49-44            | 42.6 | 229                |
| 7718-5A            | 1/16" from surface  | 37-42-41-41            |      |                    |

The foregoing data with respect to Heat Nos. 7718, 7719, and 7773 is graphically reproduced in Figure 7 from which it will be apparent that Heat No. 7773 produced a steel alloy which was much tougher than that of the other two heats.

*Example No. 3*

A basic lined induction furnace heat was produced in accordance with the following table:

| Heat No. | C   | Mn   | Si  | P    | S    | Cr  | Mo  | Ni  | B     |
|----------|-----|------|-----|------|------|-----|-----|-----|-------|
| 9203     | .30 | 1.42 | .40 | .010 | .016 | .64 | .54 | .27 | .0026 |

The steel alloy was treated in the molten state by adding 1½ pounds of aluminum per ton, then .0026% boron added as "Borosil," then 2 pounds of the rare earth metal mixture per ton, and finally 3 pounds of calcium-manganese-silicon per ton.

Runners cast from this heat were normalized by air cooling from 1750° F. after a two hour hold at temperature. The runners were then hardened by heating to 1650° F. followed by a water quench after one hour hold at temperature and were then tempered for two hours by heating to various temperatures followed by a water quench. The tempering temperatures used were selected to give a hardness range from 250 to 500 Brinell in increments of approximately 50 points Brinell. All pull bar specimens were aged for 24 hours at 250° F. The following table lists the mechanical properties of castings obtained from this heat:

| Heat No. | Serial No. | Tempering Temperature, °F. | Yield Strength (p. s. i.) | Tensile Strength (p. s. i.) | Elongation, Per cent | Red. of Area, Per cent | Charpy Impact, Ft. Lbs. |         | BHN |
|----------|------------|----------------------------|---------------------------|-----------------------------|----------------------|------------------------|-------------------------|---------|-----|
|          |            |                            |                           |                             |                      |                        | Rm. T.                  | -40° F. |     |
| 9203     | 1          | 250                        | 198,750                   | 248,500                     | 10.0                 | 31.5                   | 18-17                   | 13-16   | 514 |
|          | 2          | 250                        | 219,000                   | 246,000                     | 9.5                  | 29.8                   | 17-17                   | 15-15   | 514 |
|          | Average    | 250                        | 208,875                   | 247,250                     | 9.75                 | 30.7                   | 17.25                   | 14.75   | 514 |
|          | 3          | 350                        | 195,000                   | 239,500                     | 9.5                  | 31.2                   | 17-16                   | 16-17   | 495 |
|          | 4          | 350                        | 195,000                   | 235,500                     | 9.0                  | 30.2                   | 18-19                   | 16-16   | 495 |
|          | Average    | 350                        | 195,000                   | 237,500                     | 9.25                 | 30.7                   | 17.25                   | 16.25   | 495 |
|          | 5          | 550                        | 195,000                   | 224,000                     | 9.5                  | 31.8                   | 12-13                   | 13-9    | 444 |
|          | 6          | 550                        | 195,000                   | 234,500                     | 10.0                 | 29.8                   | 11-12                   | 13-13   | 444 |
|          | Average    | 550                        | 195,000                   | 224,250                     | 9.75                 | 30.8                   | 12.00                   | 12.00   | 444 |
|          | 7          | 750                        | 188,000                   | 204,500                     | 11.0                 | 33.8                   | 14-14                   | 10-10   | 429 |
|          | Average    | 750                        | 189,000                   | 204,500                     | 10.5                 | 33.8                   | 15-13                   | 7-10    | 429 |
|          | 9          | 950                        | 188,500                   | 204,500                     | 10.75                | 33.8                   | 14.00                   | 9.25    | 429 |
| 9203     | 10         | 950                        | 164,000                   | 177,500                     | 13.0                 | 37.0                   | 26-26                   | 16-17   | 388 |
|          | Average    | 950                        | 167,500                   | 178,000                     | 13.0                 | 35.7                   | 26-27                   | 16-16   | 375 |
|          | 11         | 1,050                      | 165,750                   | 177,750                     | 13.0                 | 36.4                   | 26.25                   | 16.25   | 382 |
|          | 12         | 1,050                      | 150,000                   | 161,500                     | 15.0                 | 44.9                   | 35-35                   | 30-31   | 352 |
|          | Average    | 1,050                      | 149,500                   | 161,500                     | 15.5                 | 47.5                   | 36-36                   | 29-27   | 352 |
|          | 13         | 1,250                      | 149,750                   | 161,500                     | 15.3                 | 46.2                   | 35.50                   | 29.25   | 352 |
|          | 14         | 1,250                      | 99,000                    | 117,000                     | 21.0                 | 58.1                   | 63-65                   | 57-59   | 248 |
|          | Average    | 1,250                      | 100,000                   | 119,000                     | 21.5                 | 57.0                   | 69-65                   | 65-66   | 255 |
|          | 15         | 1,250                      | 99,500                    | 118,000                     | 21.3                 | 57.6                   | 65.50                   | 61.75   | 252 |

The data of the foregoing table in connection with Heat No. 9203 is presented graphically in Figure 8, which emphasizes the effect of tempering temperature on the mechanical properties of the steel alloy. It may be noted

in increments of about 50 points Brinell hardness. All pull bars were aged for 24 hours at 250° F. The following table lists the mechanical properties obtained from this heat:

| Heat No. | Serial No. | Tempering Temperature, °F. | Yield Strength (p. s. i.) | Tensile Strength (p. s. i.) | Elongation, Per cent | Red. of Area, Per cent | Charpy Impact, Ft. Lbs. |         | BHN |
|----------|------------|----------------------------|---------------------------|-----------------------------|----------------------|------------------------|-------------------------|---------|-----|
|          |            |                            |                           |                             |                      |                        | Rm. T.                  | -40° F. |     |
| 9156     | 1          | 250                        | 181,500                   | 228,000                     | 9.0                  | 32.1                   | 27-22                   | 23-20   | 461 |
|          | 2          | 250                        | 183,000                   | 230,500                     | 9.0                  | 33.4                   | 24-24                   | 22-25   | 461 |
|          | 3          | 250                        | 182,250                   | 229,250                     | 9.0                  | 32.8                   | 24.3                    | 22.5    | 461 |
|          | 4          | 400                        | No Bar                    | No Bar                      | No Bar               | No Bar                 | 27-26                   | 27-23   | 444 |
|          | Average    | 400                        | 186,500                   | 228,000                     | 11.5                 | 35.0                   | 20-27                   | 22-24   | 444 |
|          | 5          | 400                        | 186,500                   | 228,000                     | 11.5                 | 35.0                   | 25.0                    | 24.0    | 444 |
|          | 6          | 800                        | 180,000                   | 188,000                     | 11.5                 | 35.7                   | 19-21                   | 17-16   | 388 |
|          | Average    | 800                        | 182,500                   | 190,000                     | 9.5                  | 27.8                   | 21-20                   | 13-12   | 388 |
|          | 7          | 1,025                      | 180,000                   | 188,000                     | 11.5                 | 35.7                   | 20.3                    | 14.5    | 388 |
|          | 8          | 1,025                      | 161,000                   | 167,500                     | 13.5                 | 43.1                   | 38-36                   | 22-22   | 358 |
|          | Average    | 1,025                      | 157,000                   | 168,000                     | 13.5                 | 41.6                   | 39-39                   | 22-23   | 358 |
|          | 9          | 1,175                      | 159,000                   | 167,750                     | 13.5                 | 42.4                   | 38.0                    | 22.3    | 358 |
|          | 10         | 1,175                      | 109,000                   | 126,500                     | 19.0                 | 56.0                   | 64-67                   | 64-60   | 269 |
|          | Average    | 1,175                      | 110,000                   | 126,500                     | 21.5                 | 57.5                   | 66-64                   | 58-60   | 269 |
|          | 11         | 1,250                      | 109,500                   | 126,500                     | 20.3                 | 56.8                   | 65.3                    | 60.5    | 269 |
|          | 12         | 1,250                      | 95,500                    | 115,000                     | 22.0                 | 58.8                   | 76-78                   | 72-72   | 241 |
|          | Average    | 1,250                      | 95,500                    | 115,500                     | 23.0                 | 55.2                   | 78-75                   | 71-72   | 241 |

<sup>1</sup> Defective bar. Not included in average data for Figure 9.

that tests at -40° F. disclosed a brittle zone for the samples tempered at 700° F., and the samples tempered at 550° F. or less were much tougher at -40° F. than those tempered at temperatures between 600 and 800° F. Furthermore the Brinell hardness of samples tempered above 700° F. indicate unsatisfactory resistance to wear.

*Example No. 4*

A 200 pound basic induction furnace heat of the novel steel alloy having the composition shown in the following table was produced in the usual manner:

| Heat No. | C   | Mn   | Si  | P    | S    | Cr   | Mo  | Ni  | B     |
|----------|-----|------|-----|------|------|------|-----|-----|-------|
| 15       | .24 | 1.31 | .42 | .009 | .018 | 1.03 | .58 | .95 | .0027 |

The heat was deoxidized by adding 1½ pounds of aluminum per ton. Following the deoxidization, 2 pounds of the rare earth metal mixture per ton and .0027% boron in the form of "Borosil" were added. Finally 3 pounds of calcium-manganese-silicon per ton were added.

Runners cast from this heat were normalized by heating to 1750° F. After a two hour hold at temperature, the runners were softened at 1250° F. for two hours and were then air cooled. The runners were then water quenched from 1650° F. after a one hour hold at temperature and were then tempered by holding for two hours at various temperatures followed by a water quench. The tempering temperatures used were selected to give a hardness range from approximately 250 to 450 Brinell

The effect of the tempering temperatures on the physical properties of the novel steel alloy is graphically depicted in Figure 9, wherein it will be seen that tempering temperatures below 700° F. resulted in specimens having a Brinell hardness of 400 or more and having Charpy values of 20 or more foot pounds at room temperature and 15 or more foot pounds at -40° F. Tempering temperatures substantially above 700° F. resulted in inadequate resistance to abrasion because of the low Brinell hardness values shown in Figure 9. At -40° F. a brittle zone resulted from tempering temperatures above 700° F. and below 900° F. The brittle zone at room temperature was not so pronounced in the case of this heat; however, it is noted that the lowest Charpy values at room temperature occurred for specimens tempered at temperatures between 600 and 750° F. As above noted, tempering temperatures below 700° F. resulted in satisfactory Charpy values at room temperature and at -40° F. and also resulted in satisfactory Brinell hardness of 400 or more.

Specimens cast from this heat and tempered at values between 250 to 500° F. were unusually excellent in that Charpy values at room temperature and at -40° F. were 20 or more foot pounds and Brinell hardness values were 430 or higher.

*Example No. 5*

Three 200 pound induction furnace heats were poured having the following analyses:

| Serial No. | Heat No. | C   | Mn   | Si  | P    | S    | Cr  | Mo  | Ni  | B     |
|------------|----------|-----|------|-----|------|------|-----|-----|-----|-------|
| 25         | 8958     | .35 | 1.42 | .39 | .010 | .013 | .65 | .50 | .27 | .0025 |
| 26         | 8958     | .35 | 1.42 | .39 | .010 | .013 | .65 | .50 | .27 | .0025 |
| 27         | 8959     | .35 | 1.42 | .41 | .010 | .014 | .64 | .50 | .28 | .0021 |
| 28         | 8959     | .35 | 1.42 | .41 | .010 | .014 | .64 | .50 | .28 | .0021 |
| 30         | 8960     | .35 | 1.44 | .41 | .011 | .011 | .64 | .50 | .27 | .0022 |

The deoxidation practice and the additions of rare earth metals and boron, and calcium-manganese-silicon were substantially the same as those discussed in connection with previous heats.

Five dipper teeth castings were poured from these heats and were normalized by heating to 1750° F. and holding for two hours followed by air cooling. The hardening treatment consisted of heating the teeth to 1650° F. with a one hour hold at this temperature. This was followed by a water quench until the castings were at a temperature of about 200° F. The castings were then reheated to the tempering temperature of about 400° F. with a two hour hold, again followed by a water quench. Brinell hardness readings were taken on the cope side of each casting with the following results:

| Casting, Serial No.: | Brinell |
|----------------------|---------|
| 25                   | 534     |
| 26                   | 534     |
| 27                   | 540     |
| 28                   | 534     |
| 30                   | 534     |

These castings were utilized in conventional dipper buckets and were subjected to trial service in the mining of taconite ore, an unusually severe type of service in which prior art teeth were worn to a condition which required replacement after service of about 300 truck loadings. The novel steel alloy teeth did not require replacement prior to 533 truck loadings and were ultimately removed to prevent wearing on a new, wider tooth holder placed in service after the novel teeth had been submitted for tests. According to conservative estimates, approximately 100 additional truck loadings would have been possible if the novel steel alloy teeth had been in use for the full service life thereof.

After removal of these novel steel alloy teeth, visual examination thereof indicated no evidence of spalling, cracking, or bending, and a slight amount of metal flow

was observed on the edges of both faces and on the edges of the holder sockets on the sides of the novel teeth indicating ductility thereof, even at the high hardness values above described.

Microscopic examination of the teeth after removal from service disclosed a hard white layer of untempered martensitic structure created by heating the surface to its upper critical temperature of about 1500° F. and subsequent rapid cooling, due to the service conditions to which the teeth were subjected. Beneath this layer the teeth were formed of the low tempered martensitic structure illustrated in Figure 5.

*Example No. 6*

Ten steel alloy dipper teeth were cast from a heat having the following composition:

| Heat No. | C   | Mn   | Si  | P    | S    | Cr  | Mo  | N   | B     | W    |
|----------|-----|------|-----|------|------|-----|-----|-----|-------|------|
| 6784     | .25 | 1.33 | .28 | .021 | .013 | .68 | .55 | .04 | .0018 | .003 |

The heat was killed in the furnace by adding ferro-manganese in an amount sufficient to bring the manganese content about equal to that stated above. The following additions were then made in the ladle: ferro-silicon in an amount to increase the silicon content to about .28, then 3 pounds of aluminum per ton of charge, then 1 pound of high carbon ferrotitanium per ton of charge, then 1½ pounds of the above described rare earth metal mixture per ton of charge, then .0035 percent by weight of boron in the form of "Borosil" and finally four pounds of calcium-manganese-silicon per ton of charge.

The castings were normalized by heating to about 1750° F. with a two hour hold at that temperature followed by air cooling to about room temperature. The castings were then hardened by heating them to about 1650° F. with a one hour hold at that temperature followed by a four minute hold in air at room temperature and then a water quench to about 150-200° F. The castings were then immediately placed into a tempering furnace and heated to about 300° F. with a two hour hold at that temperature followed by a water quench to room temperature.

These teeth had a service life of about 913 truck loadings as compared with the average of 300 truck loadings for prior art teeth. Brinell hardness readings were taken on two of the teeth before and after removal from service with the following results:

| Tooth No. | Before Shipping | After Service |
|-----------|-----------------|---------------|
| 55        |                 |               |
| 104       | 460             | 461           |
| 110       |                 | 461           |

It will be understood that certain of the following claims recite certain percentages of the rare earth metals; however, it will be understood that the exact amount of such metals in the casting cannot be accurately measured and the amounts stated in the claims refer to the residue from the treatment of the molten metal with the amounts of rare earth metals recited by the claims. It is also noted that the term "iron" in the claims includes residual impurities in ordinary amounts, such as, for example, aluminum, titanium, calcium, copper, lead, tin and others.

We claim:

1. A steel alloy casting composed of: about .20 to .50% C, about .15 to 2.5% Mn, about .1 to 2.00% Si, nil to about .025% P, nil to about .025% S, about .50 to 1.50% Cr, about .05 to .70% Mo, residual to 1.00% Ni, about .0005 to .005% B, about .0015 to 0.5%

rare earth metals, the balance—iron, said casting having an internal structure produced by normalizing at 1600 to 1900° F. followed by air cooling, then heating to about 1500 to 1650° F. followed by a quench, then heating to about 200 to less than 600° F. followed by another quench, and said casting being characterized by the properties of a Brinell hardness value of at least 444, and a Charpy impact value of at least 12 foot pounds at  $-40^{\circ}$  F.

2. A steel alloy casting composed of: about .20 to .50% C, about .15 to 2.5% Mn, about .1 to 2.00% Si, nil to about .025% P, nil to about .025% S, about .50 to 1.50% Cr, about .05 to .70% Mo, residual to 1.00% Ni, about .0005 to .005% B, about 0.0015 to 0.5% rare earth metals, about .0005 to .02% Ti, the balance—iron, said casting having an internal structure produced by normalizing at 1600 to 1900° F. followed by air cooling, then heating to about 1500 to 1650° F. followed by a quench, and then heating to about 200 to less than 600° F. followed by another quench, and said casting being characterized by the properties of a Brinell hardness value of at least 444, and a Charpy impact value of at least 12 foot pounds at  $-40^{\circ}$  F.

3. A steel alloy casting composed of: about .20 to .50% C, about .15 to 2.5% Mn, about .1 to 2.00% Si, nil to about .05% P, nil to about .05% S, nil to about 5.00% of the group consisting of Cr, Mo, and W, nil to about 4.00% Ni, about .0005 to .005% B, about 0.0015 to 0.5% rare earth metals, the balance—iron, said casting having a Brinell hardness value of 444 or more and having a Charpy impact value of at least 12 foot pounds at  $-40^{\circ}$  F.

4. A steel alloy casting composed of: about .20 to .50% C, about .15 to 2.5% Mn, about .1 to 2.00% Si, nil to about .05% P, nil to about .05% S, nil to about 5.00% of the group consisting of Cr, Mo, and W, nil to about 4.00% Ni, about .0005 to .005% B, about 0.0015 to 0.5% rare earth metals, about .0005 to .02% Ti, the balance—iron, said casting having a Brinell hardness value of 444 or more and having a Charpy impact value of the order of at least 12 foot pounds at  $-40^{\circ}$  F.

5. A steel alloy casting composed of: about .20 to .50% C, about 1.35 to 1.55% Mn, about .1 to 2.00% Si, nil to about .020% P, nil to about .020% S, about .52 to .68% Cr, about .47 to .53% Mo, Ni in residual amount, about .0005 to .005% B, about 0.0015 to 0.5% rare earth metals, the balance—iron, said casting being characterized by an internal structure having plainly visible martensitic needles produced by a heat treatment at about 1600–1900° F., then air cooling, then another heat treatment at about 1500–1700° F., followed by a quench, and then a tempering heat treatment at about 100–400° F. followed by another quench, and said casting being characterized by the properties of Brinell hardness of about 444 or more and a Charpy impact value of the order of 15 foot pounds or more at  $-40^{\circ}$  F.

6. A steel alloy casting composed of: about .20 to .50% C, about 1.55 to 1.75% Mn, about .1 to 2.00% Si, nil to about .020% P, nil to about .020% S, about .70 to .90% Cr, about .47 to .53% Mo, Ni in residual amount, about .0005 to .005% B, about 0.0015 to 0.5% rare earth metals, the balance—iron, said casting being characterized by an internal structure having plainly visible martensitic needles produced by a heat treatment at about 1600–1900° F., then air cooling, then another heat treatment at about 1450–1650° F., followed by a quench, and then a tempering heat treatment at about 200–600° F., followed by a quench, and said casting being characterized by the properties of a Brinell hardness of about 444 or more and a Charpy impact value of the order of 12 or more foot pounds at  $-40^{\circ}$  F.

7. A steel alloy casting composed of: about .20 to .50% C, about 1.25 to 2.5% Mn, about .1 to 2.00% Si, nil to about .020% P, nil to about .020% S, about .90

to 1.10% Cr, about .50 to .65% Mo, about .90 to 1.10% Ni, about .0005 to .005% B, about 0.0015 to 0.5% rare earth metals, the balance—iron, said casting having an internal structure produced by a hardening heat treatment at about 1500–1700° F. followed by a quench, and then a tempering heat treatment at about 200–600° F. followed by another quench, and said casting having the properties of a Brinell hardness of about 444 or more and a Charpy value of about 15 foot pounds at  $-40^{\circ}$  F.

8. A steel alloy casting composed of: about .20 to .50% C, about .15 to 2.5% Mn, about .1 to 2.00% Si, nil to about .020% P, nil to about .020% S, about .1 to 2.5% Cr, about .05 to 2.5% Mo, about 0 to 4.0 Ni, about .0005 to .005% B, about 0.0015 to 0.5% rare earth

metals, about .0005 to .02% Ti, the balance—iron, said casting having an internal structure produced by a normalizing heat treatment at about 1600–1900° F., followed by air cooling, then a hardening heat treatment at about 1450–1700° F., and then a tempering treatment at about 200–600° F. followed by another quench and having the property of a Brinell hardness value greater than about 444.

9. A steel alloy casting composed of: about .35 to .50% C, about 1.35 to 2.5% Mn, about .1 to 2.00% Si, nil to about .020% P, nil to about .020% S, about .60 to 2.5% Cr, about .45 to 2.5% Mo, about 0 to about 4.0% Ni, about .0005 to .005% B, about 0.0015 to 0.5% rare earth metals, the balance—iron, said casting having an internal structure produced by a normalizing heat treatment at about 1600–1900° F. followed by air cooling, then a hardening heat treatment at about 1450–1700° F. followed by a quench, and then a tempering heat treatment at about 200–600° F. followed by another quench, and said casting having a Brinell hardness value of at least about 500.

10. A steel alloy casting composed of: about .20 to .5% C, about 1.25 to 1.40% Mn, about .1 to 2.00% Si, nil to about .020% P, nil to about .020% S, about .70 to 1.05% Cr, about .50 to .65% Mo, about .90 to 1.00% Ni, about .0005 to .005% B, about 0.0015 to 0.5% rare earth metals, the balance—iron, said casting having an internal structure produced by a hardening heat treatment at about 1600–1700° F. followed by a quench, and then a tempering heat treatment at about 200–600° F. followed by another quench, and said casting having a Brinell hardness of at least about 444.

11. A steel alloy casting composed of: about .20 to .5% C, about .15 to 2.5% Mn, about .1 to 2.00% Si, nil to about .020% P, nil to about .020% S, about .70 to 1.05% Cr, about .50 to .65% Mo, about .90 to 1.00% Ni, about .0005 to .002% B, about 0.0015 to 0.5% rare earth metals, about .0005 to .02% Ti, the balance—iron, said casting having an internal structure produced by a hardening heat treatment at about 1600–1700° F. followed by a quench, and then a tempering heat treatment at about 200–600° F. followed by another quench, and said casting having a Brinell hardness of at least about 444.

12. A steel alloy casting composed of: about .20 to .5% C, about 1.30 to 1.60% Mn, about .1 to 2.0% Si, nil to about .05% P, nil to about .07% S, about .50 to .70% Cr, about .40 to .60% Mo, Ni in residual amount, about .0005 to .005% B, about 0.0015 to 0.5% rare earth metals, the balance—iron, said casting being characterized by an internal structure having plainly visible martensitic needles produced by a heat treatment at about 1500–1700° F., followed by a quench, and then a tempering heat treatment at about 200–600° F., followed by another quench, and said casting being characterized by the properties of a Brinell hardness value of about 444 or more and a Charpy impact value of the order of 15 or more foot pounds at  $-40^{\circ}$  F.

13. A steel alloy casting composed of: about .20 to .5% C, about 1.30 to 1.60% Mn, about .1 to 2.0% Si, nil to about .05% P, nil to about .07% S, about .50

to .70% Cr, about .40 to .60% Mo, Ni in residual amount, about .0005 to .005% B, about 0.0015 to 0.5% rare earth metals, the balance—iron, said casting being characterized by an internal structure having plainly visible martensitic needles produced by a heat treatment at about 1500–1700° F., followed by a quench, and then a tempering heat treatment at about 200–600° F., followed by another quench, and said casting being characterized by the properties of a Brinell hardness value of about 444+ or more and a Charpy impact value of the order of 20 or more foot pounds at –40° F.

14. In a method of treating molten steel in a basic condition, the steps of first deoxidizing the steel and reducing soluble nitrogen in the steel to a value not substantially greater than the order of about .008% by adding titanium in an amount of the order of .0005 to .02% and then, irrespective of sequence, adding boron in an amount of the order of .0005 to .005% and rare earth metals in an amount of the order of 0.0015 to 0.5%. 20

15. In a method of producing wear resisting steel, the steps of killing a bath of molten basic steel comprising: about .20 to .50% C, about .15 to 2.5% Mn, about 0.1 to 2% Si, nil to about .05% P, nil to about .07% S, nil

to about 5.00% of one or more of the group consisting of Cr, Mo, and W, nil to about 4% Ni, the balance—iron, pouring the metal into the ladle and while pouring, making the following additions in the order specified: ferro-manganese and/or ferrosilicon and about 1 to 5 pounds of aluminum per ton of charge, then adding titanium in an amount of about .0005 to .02% of the charge and then, irrespective of sequence, adding boron in an amount of the order of .0005 to .005% of the charge and rare earth metals in an amount of the order of 0.0015 to 0.5% of the charge.

References Cited in the file of this patent

UNITED STATES PATENTS

|    |           |                |               |
|----|-----------|----------------|---------------|
| 15 | 2,528,867 | Day            | Nov. 7, 1950  |
|    | 2,542,220 | Urban          | Feb. 20, 1951 |
|    | 2,586,041 | Hodge et al.   | Feb. 19, 1952 |
|    | 2,683,662 | Tisdale et al. | July 13, 1954 |

OTHER REFERENCES

Transactions, American Society for Metals, vol. 28, page 618. Published in 1940 by the American Society for Metals, Cleveland, Ohio.